

Feb. 17, 1925

1,526,492

G. H. DAVIS

MOLDED LAMINATED ARTICLE

Filed Sept. 29, 1922

*Fig. 1.*



*Fig. 2*



George Howlett Davis,  
Inventor  
By Prentiss, Stone & Boyden,  
Attorneys.

## UNITED STATES PATENT OFFICE.

GEORGE HOWLETT DAVIS, OF ORANGE, NEW JERSEY.

## MOLDED LAMINATED ARTICLE.

Application filed September 29, 1922. Serial No. 591,300.

*To all whom it may concern:*

Be it known that I, GEORGE HOWLETT DAVIS, a citizen of the United States, residing at Orange, in the county of Essex and State of New Jersey, have invented certain new and useful Improvements in Molded Laminated Articles, of which the following is a specification.

This invention relates to molded laminated articles, and more particularly to articles formed of a plurality of sheets of fibrous material, such as paper or cardboard. While the invention is particularly applicable to and will be described as embodied in a phonograph record, it is equally applicable to other articles.

Numerous attempts have heretofore been made to produce a satisfactory phonograph disc record having a body formed of fibrous material, such as paper or the like, but records of this character heretofore produced have been subject to the grave defect that they tend to warp and become distorted out of a true plane. As is obvious, such warping renders the record commercially valueless.

This warping or distortion of records with a paper base is largely due to the absorption of moisture by the paper stock and its consequent uneven expansion. Moreover, the coefficient of expansion of the paper body is often different from that of the veneering of thermoplastic material with which the body is covered and which carries the impression of the sound waves, such variation in the coefficients of expansion having a further tendency to cause warping or twisting of the record.

The primary object of the present invention, therefore, is to prevent such warping or twisting, and to provide a disc record or like article which will remain perfectly flat and true indefinitely, under all atmospheric conditions.

Phonograph disc records, as heretofore constructed, have been more or less fragile and easily broken. It is, therefore, another object of the present invention to provide a record or like article which shall be practically indestructible under ordinary handling, and which will successfully withstand shipment through the mails without elaborate protective packing. To this end, I contemplate the construction of a record or like article which shall be bendable or

flexible to a high degree, so that it will readily yield to pressure and when released, will resume its original shape.

I have discovered that the above results may be attained by building up the base or body of the record or like article from layers of paper stock of different characteristics, and particularly by employing an inner or central layer of relatively soft porous absorbent material.

In order that the invention may be more clearly understood, reference is had to the accompanying drawing, forming part of this specification, and in which:

Fig. 1 is a transverse central section through a record constructed in accordance with the preferred form of my invention; and

Fig. 2 is a similar view showing a somewhat modified construction.

Referring to the drawings in detail, I construct my improved record or similar article as follows. I first take a disc or sheet of soft, flexible, absorbent, porous, fibrous material 1, such as blotting paper. To each side of this central layer or core, I next glue or cement a disc or layer 2 of a harder, denser and less porous, fibrous material such as cardboard. The particular grade of cardboard which I have found in practice to be especially suitable for this purpose, is that known in the trade as "pattern board", and both this and the central core are preferably about two hundredths of an inch in thickness. The glue or cement which I preferably employ for uniting the central core to these outer layers is of such a nature as not to penetrate or impregnate the paper to any substantial extent, so that the central layer or core retains, to a large degree, its soft, porous and absorbent properties.

The outer surfaces of the dense outside layers 2 are preferably well calendered so that they are smooth and compact. This is desirable in order that they may not absorb too large a quantity of the thermoplastic veneering which is applied to them.

This thermoplastic veneering or surface coating is designated by the reference numeral 3, and may consist of suitable mixtures of shellac and china clay, or other well known materials usually employed in the manufacture of this type of phonograph records. This material is applied by either dusting or painting on, and the sound wave

record is impressed therein by means of a heated die.

I have found that a record constructed as above described will maintain its flat true shape indefinitely, regardless of atmospheric conditions. I believe that this is due to the fact that the central layer or core of porous, fibrous material serves to absorb whatever moisture may permeate the coating of thermoplastic material and thus serves to prevent appreciable expansion of the denser outer layers of cardboard. Moreover, the two outer layers, being disposed symmetrically, one on each side of the central absorbent layer, tend to balance each other and thus one aids in neutralizing any tendency of the other to warp. Furthermore, I preferably choose the fibre of the cardboard discs 2 in such a way that they will have a minimum coefficient of expansion and that such coefficient shall be as nearly as possible equal to the coefficient of expansion of the veneering or thermoplastic coating.

25 The use of a soft, yieldable central layer or core also results in rendering the record exceptionally flexible and unbreakable in its nature. The looseness of the fibre of the central core or layer permits the outer layers to have a slight movement relative thereto and to each other, when a bending force is applied to the record, much in the same way that a slight slippage occurs between a loose package of paper sheets 30 when the package is bent. The hardness of the two outer layers of my improved record, however, causes the record to spring back into normal shape as soon as the bending pressure is relieved.

40 In Fig. 2, I have shown a slightly modified construction in which only two sheets of fibrous material are employed. These sheets are designated by the numeral 4 and are somewhat thicker than the sheets 45 shown in Fig. 1. Each of the sheets 4 is formed from stock, one side of which only is calendered or hard finished, the other side being relatively soft and porous. In forming the record body, the two sheets are placed with their rough porous faces together, and are united by a suitable glue or cement which is of such a nature as not to impregnate the paper to any substantial extent. A coating of thermoplastic veneering 55 3 is then applied to the outer calendered surfaces of the sheets 4, in the usual way.

From the above described method of manufacture, there results a structure having a central portion which is of a loose porous absorbent nature, and outer portions of a harder, denser and more compact character. In this way, a record having much the same characteristics as that shown in Fig. 1 is produced.

60 It will thus be seen that the essential

feature of my improved record or like article consists in the provision of a central layer or core of soft, flexible, absorbent material, and that a record constructed in accordance with my invention is both free 70 from any tendency to warp and is bendable and substantially indestructible with any ordinary handling, and it is thought that the many advantages of my improved article will be readily appreciated without 75 further discussion.

What I claim is:

1. A molded article having a central core of relatively loose porous material, superposed layers of denser, more compact 80 fibrous material, and a surface coating of thermoplastic material.

2. A laminated structure having a body built up of assembled layers of fibrous material, the central portion of said body being 85 softer and more porous than the outer portions thereof, and a surface coating of thermoplastic material on said body.

3. A laminated structure having a body formed of assembled sheets, and a surface 90 layer of thermoplastic material on said body, the inner portion of said body being of a loose, fibrous nature and more absorbent than the outer portions thereof.

4. A laminated structure having a body formed of assembled sheets of fibrous material, and a surface coating of plastic material on said body, the inner portion of said body being of a loose, soft nature and more porous and absorbent than the outer 100 portions thereof.

5. A molded article having a central core of relatively soft, porous, unimpregnated fibrous material, a layer of inherently denser, less porous, stiff fibrous material on 105 each side of said core, and a surface coating of plastic material.

6. A molded article comprising a central sheet of porous flexible paper of soft, loose texture, a stiff sheet of denser and less porous paper cemented to each side of said central sheet, and a thin coating of plastic material covering said denser sheets.

7. A molded article comprising a central sheet of porous flexible paper, a stiff sheet 115 of denser and less porous paper cemented to each side of said central sheet, and a thin coating of plastic material covering said denser sheets, the outer surface of said denser sheets to which the coating is applied 120 being calendered.

8. A laminated article comprising a porous central sheet of loose fibrous material, a relatively dense sheet cemented to each side of the porous sheet, and a suitable 125 surface coating on said outside sheets.

9. A molded article comprising a sheet of soft, porous paper, a sheet of relatively hard dense paper cemented to each side of said central sheet, the outer surfaces of said 130

dense paper being smooth calendered, and a thermoplastic veneer applied to said smooth calendered surfaces.

10. A laminated phonograph record having an inner layer of permanently soft yielding material to which outer fibrous layers are cemented, whereby the structure is rendered flexible.

11. A laminated phonograph record having an inner layer of soft yielding material, outer layers of relatively dense stiff material

cemented to the interior layer, and a veneering of thermoplastic material on said outer layers, the inner layer being united to the adjacent layers by a cement which does not impregnate its surface to any substantial extent, whereby sufficient relative movement of said outer and inner layers is permitted to render said record flexible.

In testimony whereof I affix my signature.

GEORGE HOWLETT DAVIS.